

March 16, 1937.

F. H. WILLEY

2,074,038

DIAMOND EMBEDDED ABRADING TOOL

Filed May 29, 1935

2 Sheets-Sheet 1



INVENTOR.  
Fay H. Willey.  
BY  
Gerald E. Willey  
ATTORNEY.

March 16, 1937.

F. H. WILLEY

2,074,038

DIAMOND EMBEDDED ABRADING TOOL

Filed May 29, 1935

2 Sheets-Sheet 2



INVENTOR.

Fay H. Willey.

Charles E. Wilson

ATTORNEY.

## UNITED STATES PATENT OFFICE

2,074,038

## DIAMOND EMBEDDED ABRADING TOOL

Fay H. Willey, Detroit, Mich.

Application May 29, 1935, Serial No. 24,068

12 Claims. (Cl. 51—280)

This invention relates to abrading, drilling or surfacing tools, the object being to provide an improved abrading tool or tip for tools of a hard and tough metal alloy in which a diamond or diamonds of various sizes may be embedded to form abrading or surfacing tools, the composition being of such character that the diamonds are so securely seated in the alloy as to prevent displacement or unseating by pressures or impact less than that causing fracture of the diamond and thus provide a more highly efficient abrading tool and one of longer life than has heretofore been secured.

The invention also has for its object to provide an improved process for the formation of such tool whereby the surfaces of the diamonds give up carbon to the alloy and thus unite the diamond and the alloy as distinguished from a mere adhesion or "wetting" of the diamond surface by the metal as has heretofore been the method in this art.

A feature of the invention is involved in the formation of a diamond abrading or cutting tool by heating powdered tungsten (W), carbon (C), and nickel (Ni) to alloying temperature, the carbon content being insufficient to satisfy the tungsten and the diamonds being distributed therethrough; the heating, as hereinafter described, being step by step under pressure to a final temperature of the order of 1700 degrees C. while occluded to atmosphere to prevent oxidation and for a short period of time sufficient to cause the surfaces of the diamonds only to gasify and combine with the tungsten to form a tungsten-carbide seat in cohesive relation with the diamond.

It has heretofore been proposed to form an abrading and surfacing tool by mixing diamond dust and diamond particles in a material such as powdered tungsten-carbide and submitting to a sintering temperature. My improved tool distinguishes from such former tools in that the diamonds used are not what is known to the trade as diamond dust or diamond particles but are true diamonds usually, by way of example but not of limitation, more than one-sixteenth of an inch across the surface in any direction and ordinarily nearly one-eighth of an inch and oftentimes with diamonds of such size, there is incorporated a diamond at the very tip of the tool materially greater in size surrounded by the smaller diamonds.

While, in general, the invention is not limited to the size of the diamonds yet it is pointed out

that, with such sizes as have been suggested, I am enabled to bring the metals to an alloying temperature for a few seconds of time without loss of the diamond as apparently only the surface of the diamonds becomes affected sufficiently to permit the carbon at the surface to be taken up by the tungsten and thus provide what may be termed an integral seat; that is an actual cohesion between the diamond and the metal rather than a mere adhesion therebetween as is the result at sintering temperature of approximately 1350° C.

It is further an object of the invention to provide a new and improved process for the manufacture of a tool of the character stated which consists in the placing of a graphite or graphite lined mold having a recess of the desired depth and shape in cross section between the electrodes of a welding machine, placing a small quantity of the powdered tungsten, carbon, and nickel with diamonds in the cavity, tamping the same, adding in succession small quantities of the powdered material and diamonds, each charge being tamped in succession until a body of the compacted powder and diamonds of the desired length is secured, then, while light pressure is applied and the material occluded to atmosphere, heating the mold and the prepared material to a sufficiently high temperature approximately 800 degrees C. to start gas formation and discharge of included air and also, due to the pressure, increasing the density or compactness, then increasing the temperature and pressure in successive steps or stages until finally a temperature of the order of 1700 degrees C. and a final pressure of approximately 10,000 pounds per square inch is attained for a period less than that productive of liquefaction of the metals.

By the above described manner of compacting the material and heating in successive stages under increasing temperature and pressure, the voids usually occurring in the material at sintering temperature are prevented and an actual alloy of the metals in a plastic state is secured.

The process therefore distinguishes from former processes wherein the material may be compacted under pressure in a mold and then with the mold, or even removed from the mold, placed in a furnace and brought to sintering temperature. By my improved process the tool is completed in the welding machine, first using the machine and the ram or plunger to tamp and compact the material and then to apply the pressure under the heat in the successive stages, as before mentioned, and at the final heat, the article is completely formed

requiring only removal from the mold and the surface cleaned. The process is therefore more rapid than former processes of which I have any knowledge, is of less labor cost and a more serviceable tool is secured due to the density of the product and the seating of the diamonds in place which are so solidly secured that fracture will occur along the cleavage plane of the diamond before it can be loosened.

10 These and other desirable objects and features of the invention are hereinafter more fully described and claimed, it being understood that the specific embodiments of the invention described are by way of illustration and not of limitation 15 as the methods involved and the components of the alloy may be varied considerably without departing from the spirit and scope of the invention.

In the accompanying drawings:

20 Fig. 1 is a side elevation partly in section of an electric welding machine suitable for manufacture of my improved tool or tip.

Fig. 2 is a section taken on line 2—2 of Fig. 1.

25 Fig. 3 is an elevation taken from the right hand side of Fig. 1.

Fig. 4 is an enlarged section showing a graphite lined mold with the formed tip therein.

30 Preferably, the invention is described in conjunction with the use of tungsten as an element 35 of the alloy but other elements that have the necessary hardness and tendency to absorb carbon may be utilized with any of the iron group such as nickel, cobalt or iron. The preferred composition is tungsten (W), carbon (C), nickel (NI), the tungsten being unsatisfied with carbon and the nickel being used to form an alloy to provide toughness and preventative of cracking or shatter of the tool through impact or shock.

40 The invention may be best understood from the following description of the method of producing the article.

45 The mechanism for producing the article may be an electric welding machine such as is shown in Fig. 1 having the water cooled electrodes 1 and 45 2. The crucible, as indicated at 3, is positioned therebetween and may rest upon a water cooled base 4. The electrode 1 is supported in a carrier 5 which is movable on the base 6 of the machine by means of a hand wheel 7, the electrode 1 being 50 retracted to permit introduction of the crucible and then moved forward by means of the screw until the crucible is held in pressure contact between the electrodes. The crucible may be carbon or graphite or a metal crucible lined with 55 carbon or graphite. In either case, the graphite element is recessed as indicated at 8 in Fig. 4 and is preferably slightly coned at the bottom 9. A vertically reciprocable plunger 10 has a molybdenum or other hard metal tip for entering the recess and is supported by the holder 11 reciprocable in the bracket 12 attached to the standard 13 which in turn is supported on the base 6. The bracket 12 supports the holder from lateral displacement and sustains it in truly vertical position. The upper end of the standard 13 has a 65 chambered head 14 secured thereto within which is a coiled spring 15. The upper end of the chambered member is threaded to receive a plug 16 having a central projection 17 engaging in the end coil of the spring and centering the same and this may be adjusted to increase or decrease the 70 normal tension on the spring.

75 At the bottom of the chambered member 14 is a spring seat 18 having a projection entering the bottom coil of the spring to center the same and

the member 18 is centrally threaded to receive a threaded sleeve 19 which is adjustable longitudinally in the spring seat 18. A stub shaft 20 extends through the sleeve and is secured in place by the nut 21. The lower end thereof is in the form of a yoke 22 which receives a plate 23 pivoted thereto by a pin 24. The opposite end of the plate is formed with a yoke 25 in which an end of the link 26 is pivoted, the opposite end being pivoted to the upper end of the holder 11 by the pin 27. To the plate is secured a handle 28. The link and plate form a toggle between the yoke 25 at the upper end and the holder 11 at the lower end and by operation of the handle, the holder and the plunger member or tamp 10 may be reciprocated. The normal position of the parts is indicated by dotted lines in Fig. 1 and when pressure is applied to the material in the crucible or mold, the handle 28 is moved downwardly as indicated by full lines in Fig. 1. In order that pressures to be applied may be determined, the screw seat 18 is provided with a finger 29 extending through a slot 30 in the chambered member 14 and a calibrated gauge plate 31 is secured to the member 14 across which the finger is movable 25 enabling the operator to determine the pressure applied by downward movement of the handle 28. The pivot pins 24 and 27 extend to one side of the leverage mechanism as shown in Fig. 3, and a coiled spring 32 is attached thereto tending normally to hold the handle up with the plunger 10 out of the recess of the crucible as shown in dotted lines in Fig. 1.

No attempt has been made to show the electric circuit for the electrodes or the means of supplying water thereto for cooling the same, such elements being usual in welding machines.

One of the purposes of use of the welding machine or like instrumentality is to enable the article to be completely formed therein. It has heretofore been the practice to compact a material and even to heat it somewhat in a machine of this character and then remove the mold or crucible and complete the temperature treatment in a furnace or to remove the material after heating sufficiently to retain its shape and subjecting it to a sintering temperature in a furnace. However, in the method hereinafter described and in order to secure a tool of the proper hardness and density, the entire treatment of the material is completed in the welding machine thus not only saving the labor cost of handling but also saving considerable equipment and permitting the tool to be completed under a high pressure while it is at a temperature above the sintering temperature and it also enables the entire process to be performed while the material is prevented from oxidation as it is occluded from atmosphere during the forming operation and also by being encased in a graphite crucible and at the temperature attained creates a reducing atmosphere. This in turn unites with the oxygen present to form carbon dioxide which is driven off as a gas by the pressure obtained thereby removing the oxide from the material.

As an instance and not by way of limitation, I form a powder containing approximately 60 to 70 per cent tungsten (W) and 3 to 5 per cent carbon (C) and the balance nickel (NI) and ball mill the same for a number of hours sufficient to produce a very fine powder. Usually the material is placed in the mill in more or less of a granular form and ball milled for upwards of 120 hours.

Where a tool having a high abrasive quality is required, diamonds are utilized and one method of

procedure in forming a tool embedded with diamonds is as follows:

A diamond of any desired size, preferably of larger size than the remainder, is first placed in the crucible in which it centers due to its having a coned seat. Additional small diamonds may be placed about this central diamond if desired. In either case, subsequent to placement of the diamond or diamonds, a small quantity of powder 5 of the above composition, or the equivalent of the above composition, is placed on the diamonds and tamped as before stated. The diamonds are protected from being broken due to the cushioning effect of the powdered material placed thereon. When the first tamping has been completed, several other small diamonds are placed on the top thereof, an additional charge of powdered material placed thereover and tamped, and thus, in several steps or stages, the material is brought 10 up to the required depth in the mold to form an article of the desired length. Subsequent to tamping, current is turned on during application of the pressure by the tamping implement 15 until at a temperature of about 800 degrees C. is attained which may be determined by color or otherwise which starts the gasification and drives off included air and then it is allowed to cool to below said temperature. Then a higher pressure is applied and current is applied until a higher 20 temperature is attained and this is repeated until the gas has been entirely driven off or absorbed and the material placed under the highest pressure and temperature.

In the method of involving the embedment 25 of the diamonds in a material, air is excluded therefrom and thus oxidation of the diamonds is prevented. The material being under high temperature and the diamonds entirely covered with the material, the surface of the diamonds will give up carbon to the tungsten to thereby form 30 a union of the diamond, tungsten and nickel. The diamond is therefore held in place by practically an integral association of the diamond, tungsten and nickel. This association is so complete that I have in many experiments attempted 35 picking the diamond out of the material but in every instance of a tool made under the high pressures and temperatures and manner herein described, it is not possible to unseat the diamond as only particles thereof will break out 40 leaving particles of the diamonds in the surface of the recess.

It is apparent from an examination of the completed article that the diamonds give up 45 carbon to the tungsten at the surface forming a thin "skin" of a very hard tungsten-carbide encasing the diamond which is readily distinguished by the unaided eye from the contiguous metal with which it is united.

I prefer to use diamonds not smaller than 50 would pass a 20-mesh screen and such diamonds, when embedded in the metal by my improved process, appear in a whole state in the finished article and apparently uninjured in structure 55 by the heat and pressure to which they have been subjected.

The method above described results in the formation of a tip of longer life than the usual sintered tungsten-carbide tools of the prior art 60 due to greater compactness, less liability of fracture and greater hardness and when employed with diamonds as in the formation of the drills or abrading tools for the trueing of the grinding wheels and such general service as is required 65 in the industrial arts, I have provided a diamond 70

75 embedded tip which, in so far as the metals are concerned, has all of the desirable qualities above mentioned in respect to the alloy and due to the inclusion of the diamonds has a higher abrading characteristic with practically no liability of diamonds becoming unseated as it is not possible to unseat the diamonds except by fracturing the same under an excessive pressure and even then they are not truly unseated. Thus the tool is 80 of a quality highly desirable in the arts as its efficiency is not destroyed by loss of diamonds in the ordinary uses to which the tool is subjected and thus may be efficiently used through a much longer period of time than the usual diamond 85 embedded tools of the prior art which are usually sintered and thus have a considerable number 90 of voids and are more brittle than a tool formed after the manner above described in which the material is actually alloyed and practically free 95 from voids.

20 It is also pointed out that the percentage of tungsten, nickel and carbon may vary somewhat even more than ten per cent above or below the percentages hereinbefore specified, and if one 25 is increased in percentage another may be reduced in percentage depending entirely upon the character of the tool to be produced. A tool less hard may be used for some operations and of greater hardness for others may be produced and this is usually secured through increasing 30 or decreasing the carbon content. With a diamond embedded tool, I prefer to use as a base a tungsten (W) and thus even though some carbon be utilized in the composition and ball milled as described, the composition still has a high 35 avidity for carbon which is a desirable characteristic in the manufacture of a diamond embedded tool. A major feature of the invention resides in the use of a high degree of pressure 40 at alloying temperature of the metals used, which temperature and pressure so far as I know, has not before been used in the manufacture of 45 diamond embedded tools of this general type.

From the foregoing description it will be realized that the charging of the crucible by successive stages with diamonds and the powdered material, provides a very compact powdered mass 50 prior to application of heat and then by heating and cooling by successive stages of increasing temperatures and pressure up to an alloying temperature and pressure of approximately 10,000 pounds per square inch, great compactness is secured and a tool having a highly carburized surface is provided and one of the extreme hardness 55 coupled with toughness preventative of fracture under normal conditions of operation and use and free from the defects of the sintered compositions of the prior art.

It is pointed out that, while tungsten and nickel 60 are the preferred materials to be used, a metal of the 6th group of Mendelejeff's periodic table may be used together with a metal of the iron group. In any case the metal of the said 6th group of Mendelejeff's periodic table should be unsatisfied as to carbon but not wholly so, it 65 being highly desirable that the metal having an avidity for carbon will, during the process, absorb carbon from the crucible and in the case of the diamond embedded tool will, at the temperatures and pressures given, tend to take carbon from the diamond surface and thus unite the diamond and the metal by what may be termed partial graphitization of the diamond. The invention 70 also is not confined to nickel as an element but it is the preferred element of the iron group and 75

in my experience is productive of the most satisfactory tool.

It is further evident from the foregoing description that major features of the invention 5 reside in the formation of an alloy of metals such as tungsten and nickel with insufficient free carbon to satisfy the tungsten, the alloying being performed while the material is occluded to atmosphere and the diamonds in place in the material; that the entire series of steps, except the ball milling to form the powder, may be performed in a single purpose machine such as the welding machine herein described, and that the completed tool or tip is characterized by carburation of the tungsten or like material in contact with the diamond or diamonds.

From the foregoing it is believed evident that the described invention, both in method and article produced, differs from the known art in 20 that tungsten having a certain avidity for carbon is first in very finely divided form compacted with diamonds of a material size which has herein been termed "whole diamonds" (—that is, not diamond dust or diamond fragments heretofore 25 in use). The compacted material is then heated, preferably by successive stages in order to eliminate included air and gases formed during the heating process, to such final temperature and high pressure that the tungsten will satisfy its 30 remaining avidity for carbon by taking the same from the diamond. If tungsten carbide be used in the process, the carbon content should first be determined in order that the remaining amount of carbon necessary to satisfy its avidity 35 therefor may be known, it being necessary that the avidity for the tungsten for carbon shall not be entirely satisfied in order that in the steps of the process an when at the necessary temperature, the tungsten will take carbon from the diamond surfaces to securely seat the diamonds in 40 the composition. I, however, prefer to use substantially pure tungsten (W) and provide the required carbon so that the avidity of the tungsten for carbon is materially less than would tend 45 to absorb the diamond. Thus in the final heating to which the material and diamonds embedded therein are subjected, only a very small "skin" surface of the diamond can combine with the tungsten. With the "whole" diamonds as 50 hereinbefore defined, there is considerable surface in close contact with the carbon covered tungsten particles and this diamond encasing portion of the material, due to carbon being taken from the diamond by the tungsten, is extremely 55 hard and has an integral relation with the diamond while between the several diamonds, the metal is softer than at the diamond seat due to lack of carbon at such points and is thus less brittle and more serviceable in use than would be 60 the case if the tungsten throughout the mass were equally saturated with carbon. There is thus less liability of the tool breaking in use and my improved tool is characterized by this extremely hard tungsten carbide seat for the diamonds and 65 the softer and less hard tungsten carbide between the diamonds.

Having thus described my improved composition and diamond embedded abrading tool and the process of producing the same, what I claim 70 and desire to secure by Letters Patent of the United States is—

1. The method of forming a diamond embedded abrasive tool for use in the industrial arts consisting in first forming and mixing together 75 a fine powder consisting of a major portion of

w tungsten having its avidity for carbon partially satisfied and the balance nickel, adding a desired quantity of whole diamonds to the powdered material, subjecting the powdered materials containing the diamonds to a temperature of in the neighborhood of 2,000 to 1700 degrees C. while occluded from atmosphere and for a period of time tending to cause the diamonds to give up carbon at the surface to combine with the tungsten and produce a tungsten-carbide seat in 10 cohering relation with the diamonds, the time period being less than that resulting in the liquefaction of the metals.

2. The method of forming a hard metal alloy suitable for tools which consists in first reducing 15 a granular composition consisting of tungsten, a quantity of carbon insufficient to satisfy the avidity of the tungsten therefor, and the balance nickel to a finely powdered form, then placing a small quantity of the powdered material in a 20 graphite mold, tamping the material to mechanically compact the same, adding successive small quantities of the material together with a number of whole diamonds and tamping each of said small quantities in succession until the proper 25 quantity of material and diamonds have been placed in the mold and tamped, then, while under a medium pressure, heating the same to about 800 degrees C. for a few seconds of time tending to cause the materials to give off gas and eliminate 30 air, then permitting the heated material to cool, then, in successive stages of increasing pressure and temperature and cooling, and finally heating the material to above 1200 degrees C. while under pressure sufficient to prevent voids.

3. The method of forming a diamond embedded abrasive tool which consists in first reducing a granular composition consisting of a major portion of tungsten therefor, a quantity of carbon insufficient to satisfy the avidity of the tungsten, and the balance nickel to a finely powdered and mixed condition, placing a small quantity of powdered material in a graphite mold, tamping the material to mechanically pack the same, placing a small number of diamonds on the compacted material, then adding an additional small quantity of material and tamping the same, then adding another small quantity of diamonds and repeating the operation until the desired length 40 of tool and desired quantity of diamonds are compacted together, then, while under a medium pressure, heating the same to about 800 degrees C. to produce a gas and drive off the included air, then permitting the heated material to cool, then 45 submitting the material to successive stages of increasing temperature and cooling the material between the stages to a final step of heating the material to above 1200 degrees C. while under pressure of the order of 50,000 pounds per square inch, the tungsten in contact with the mold surface and the surfaces of the diamonds taking up carbon therefrom to form a very hard surfaced tool and to encase the diamonds with a tungsten-carbide which is united with the diamond on the one side and with the metal on the other.

4. The method of forming a diamond embedded abrasive tool which consists in providing a thoroughly mixed and finely powdered composition consisting of a major proportion of tungsten, carbon in quantity insufficient to satisfy the tungsten, and the balance nickel, placing the material in a graphite mold together with a quantity of diamonds of a size that will pass a 20-mesh screen or larger, the mold being positioned between the 50 55 60 65 70 75

electrodes of a welding machine having a hard metal plunger adapted to enter the mold, placing a carbon button on the top of the material to shield the plunger from contact with the metals, 5 then applying an electric current to heat the material and the mold, while under a medium pressure by the plunger, to about 800 degrees C., then, in successive stages of increasing temperature and pressure and cooling therebetween, 10 finally applying a pressure of approximately 50,000 pounds to the square inch while at a temperature of the order of 2000 degrees C. to alloy the material, the tungsten taking up carbon from the diamond surfaces and forming thereabout a 15 thin case of tungsten-carbide.

5. The method of forming a diamond embedded abrasive tool which consists in first forming a fine powder of a metal such as tungsten in major quantity, carbon in quantity less than that required to satisfy the avidity of the tungsten therefor, and the remainder a metal such as nickel, 20 then mechanically compacting the powdered material with diamonds distributed therein in the cavity of a graphite mold having an opening 25 through the surface thereof for insertion of a tamping tool, and then, while under pressure applied by the tamping tool, heating the material gradually by successive stages of heating and cooling under successive increasing pressures and 30 temperature until a temperature and pressure is attained sufficient to form an alloy of the metals and to cause carburization of the tungsten particles in contact with the diamond.

6. The method of forming a diamond embedded 35 abrasive tool which consists in first forming a fine powder of a metal such as tungsten in major quantity, carbon in quantity less than that required to satisfy the avidity of the tungsten therefor, and the remainder a metal such as 40 nickel, mechanically compacting the material with diamonds distributed therein in a cavity of a graphite mold held between electrodes of a welding machine and having an opening through the surface thereof for insertion of a tamping 45 tool, then applying pressure by the tamping tool and current to the electrodes to heat the mold and the material to approximately 800 degrees C. to thereby cause the material to become further compacted and to drive off the included air, then 50 cooling the same, then in several successive stages heating under increasing temperature and pressure, and finally heating the material to in the neighborhood of 1700 degrees C. for a period of about five seconds of time to form an alloy of 55 the metals and carburization of the tungsten particles in contact with the diamond surfaces.

7. The method of providing an abrading tool or tip comprising mixing a small quantity of whole diamonds of a size that will pass a 20- 60 mesh screen with a powdered composition consisting of a metal such as tungsten about 60 to 70 per cent, carbon about 3 to 5 per cent, and the remainder a metal such as nickel, then heating the same while occluded to atmosphere through a 65 number of successive stages of heating and cooling under pressure, the first of which is at low temperature and pressure to cause discharge of the included air from the material, and the final stage at a temperature and pressure sufficient 70 to alloy the metals and to form a tungsten carbide at the surfaces of the diamonds due to avidity thereof for carbon.

8. The method of forming a diamond embedded

abrading tool consisting in first preparing tungsten with a predetermined amount of carbon less than will satisfy the avidity of the tungsten therefor, positioning whole diamonds in the said body in spaced relation, submitting the diamond embedded material to pressure and heat, attaining at the end of the heating step a temperature of the order of 1700 degrees C., and a pressure sufficiently high to prevent voids and insure intimate contact of the material with the surface of the diamonds to thereby provide a seat for the diamond surface intimately associated with the encasing tungsten of a high degree of hardness through the taking of the carbon from the diamond surface and a less brittle and hard body of 15 the material in the spaces between the diamond seats.

9. The method of forming a diamond embedded metallic composition which consists in forming a very fine powder of the following ingredients— 20 namely, a major portion of substantially pure tungsten, a quantity of carbon insufficient to satisfy the avidity of the tungsten therefor and the balance nickel, positioning a desired quantity of diamonds in spaced relation in the powdered material, and then subjecting the powdered materials and diamonds therein to a temperature approximating 1700 degrees C., for a period to cause the diamonds to give up carbon at the surface to the tungsten and produce cohesion there- 25 between, and applying a sufficiently high pressure to the material while at the high temperature to eliminate gases and prevent voids.

10. A diamond embedded abrading tool comprising a body formed of tungsten, a metal of the iron group, and carbon in quantity less than that required to satisfy the avidity of the tungsten therefor, diamonds interspersed therein in spaced relation to provide an appreciable thickness of metal between adjacent diamonds, the metal in 35 contact with the diamond surfaces forming a seat of a high degree of hardness practically integral with the diamonds and in integral relation with the metal between the diamonds of a less degree of hardness thereby providing a tool where- 40 in the metal body wears more readily than metal in contact with the diamonds.

11. A diamond embedded abrading tool comprising a body formed of tungsten in major quantity, a metal of the iron group in minor quantity, 50 and carbon in quantity less than that required to satisfy the avidity of the tungsten therefor, diamonds positioned in the composition at approximately the surface of the body and in appreciable spaced relation one from the other, the metal forming the core of the body and extending between the diamonds being of less hardness than the metal in contact with the diamond surfaces and providing a tool characterized by having a practically non-brittle metal body of less wear 55 resistant quality than the metal in contact with the diamonds.

12. A diamond embedded abrading tool comprising a body formed of tungsten, nickel and carbon, diamonds interspersed in the composition in appreciable spaced relation one from the other, the metal spacing the diamonds being of greatest hardness at the diamond surface thereby providing a tool having a metal body less wear 65 resistant than the metal in contact with the 70 diamonds.

FAY H. WILLEY.